



US007250382B2

(12) **United States Patent**  
Takai et al.

(10) **Patent No.:** US 7,250,382 B2  
(45) **Date of Patent:** \*Jul. 31, 2007

(54) **WATER-DISINTEGRATABLE SHEET AND MANUFACTURING METHOD THEREOF**

(75) Inventors: **Hisashi Takai**, Kagawa (JP); **Kazuya Okada**, Kagawa (JP); **Takayoshi Konishi**, Kagawa (JP)

(73) Assignee: **Uni-Charm Corporation**, Ehime (JP)

(\*) Notice: Subject to any disclaimer, the term of this patent is extended or adjusted under 35 U.S.C. 154(b) by 98 days.

This patent is subject to a terminal disclaimer.

(21) Appl. No.: **10/266,421**

(22) Filed: **Oct. 8, 2002**

(65) **Prior Publication Data**

US 2003/0099821 A1 May 29, 2003

(30) **Foreign Application Priority Data**

Oct. 15, 2001 (JP) ..... 2001-316697

(51) **Int. Cl.**

**D04H 1/00** (2006.01)  
**B32B 27/04** (2006.01)  
**B27N 1/00** (2006.01)

(52) **U.S. Cl.** ..... **442/414; 428/292.1; 428/300.4; 428/332; 162/91; 162/98; 162/147; 162/148**

(58) **Field of Classification Search** ..... **442/408, 442/414; 428/300.4, 292.1, 332; 162/115, 162/91, 98, 97, 99, 147, 148**

See application file for complete search history.

(56) **References Cited**

**U.S. PATENT DOCUMENTS**

5,958,186 A 9/1999 Holm et al.  
6,132,557 A \* 10/2000 Takeuchi et al. .... 162/141  
6,258,210 B1 7/2001 Takeuchi et al.  
6,602,386 B1 \* 8/2003 Takeuchi et al. .... 162/115  
6,747,186 B2 \* 6/2004 Shimizu ..... 604/364  
2002/0013559 A1 \* 1/2002 Shimizu ..... 604/364  
2003/0100240 A1 \* 5/2003 Takai et al. .... 442/408

**FOREIGN PATENT DOCUMENTS**

EP 0 033 528 A1 8/1981  
EP 0 303 528 A1 2/1989  
EP 1 084 689 A2 \* 3/2001

(Continued)

**OTHER PUBLICATIONS**

Database WPI, Section Ch, Week 199347, Derwent Publications Ltd., London, GB; Clas D22, AN 1993-375060, XP002242104 & JP 05-279985 Oct. 26, 1993, Abstract.

(Continued)

*Primary Examiner*—Lynda Salvatore

(74) *Attorney, Agent, or Firm*—Darby & Darby

(57) **ABSTRACT**

Disclosed is a water disintegratable sheet including bast/leaf fibers and at least one kind of primary fibers. The bast/leaf fibers have a Canadian Standard freeness value of at most 600 milliliter and occupy 2 to 75% by weight of a total fiber weight of the sheet.

**6 Claims, 2 Drawing Sheets**



FOREIGN PATENT DOCUMENTS

|    |                |                           |
|----|----------------|---------------------------|
| EP | 1 091 042 A1   | 4/2001                    |
| JP | 05-279985      | 10/1993                   |
| JP | 05279985 A     | * 10/1993 ..... 162/157.2 |
| JP | 09-285709 A    | 11/1997                   |
| JP | 10-140494      | 5/1998                    |
| JP | 2001-098489 A  | 4/2001                    |
| JP | 2001-172850 A  | 6/2001                    |
| WO | WO-98/31626 A1 | 7/1998                    |

OTHER PUBLICATIONS

Database WPI, Section Ch, Week 199831, Derwent Publications Ltd., London GB; An 1998-358081, XP002242105 & JP 10 140494, May 26, 1998, Abstract.

Notice of Reasons for Rejection for Japanese Patent Application No. 2001-316697 mailed on Nov. 22, 2005.

\* cited by examiner

Fig. 1



Fig. 2



## WATER-DISINTEGRABLE SHEET AND MANUFACTURING METHOD THEREOF

### INCORPORATION BY REFERENCE

The present application claims priority under 35 U.S.C. § 119 to Japanese Patent Application No. 2001-316697 filed on Oct. 15, 2001, the entire contents of which being hereby incorporated herein by reference.

### BACKGROUND OF THE INVENTION

#### 1. Field of the Invention

The present invention relates to a water disintegratable sheet of which fibers can be dispersed in a large amount of water, more particularly, relates to a water disintegratable sheet which can offer a good balance of strength and water disintegratability.

#### 2. Description of the Related Art

It is preferred that wet sheets for wiping a discharging part of a human body and wet wipers for cleaning a toilet are disintegratable in water. In absorbent articles such as sanitary napkin, panty liner and disposable diaper, it is also preferred that a topsheet covering a top surface of an absorbent layer and a backsheet covering a bottom surface of the absorbent layer are disintegratable in water. In addition, packaging sheets for packaging such absorbent articles are also preferably disintegratable in water.

If these sheets are disintegratable in water, they can be disposed of in a flush toilet after use. Such water disintegratable sheet disposed of in a flush toilet is immersed in a large amount of water in a flush toilet or a septic tank, and constituent fibers of the water disintegratable sheet are dispersed in water, thereby preventing the sheet from floating and remaining in a septic tank.

In such water disintegratable sheet, dry strength should be excellent as well as wet strength should be increased to some extent. When put in a large amount of water, on the other hand, the constituent fibers should be rapidly dispersed.

Japanese Unexamined Patent Publication No. H10-140494 (1998/140494) discloses a water disintegratable paper which is manufactured by impregnating a nonwoven fabric or paper with a pH reactive binder for increasing the strength and a pH buffer solution which is prepared with an organic acid to have an acidic pH. With the pH reactive binder, the water disintegratable paper has high strength when it has an acidic pH, so as not to disintegrate in water. When it has a neutral or alkaline pH, on the other hand, the paper is intended to disintegrate in water. In detail, when the water disintegratable paper is immersed in a large amount of water for neutralization, the binder is dissolved in water, so that fibers forming the water disintegratable paper are dispersed for disintegration of the water disintegratable paper in water.

On the other hand, Japanese Unexamined Patent Publication No. H5-279985 (1993/279985) discloses a nonwoven sheet formed only of ramie cellulose fibers. This nonwoven sheet comprises fibrillated ramie fibers and microfibrillated ramie fibers. The microfibrillated ramie fibers function as a binder for bonding the fibrillated ramie fibers to obtain sheet strength.

However, since the water disintegratable paper disclosed in Japanese Unexamined Patent Publication No. H10-140494 is impregnated with the pH reactive binder and the pH buffer solution, it may possibly exert a baneful influence upon the body of a user. In addition, when the water disintegratable paper is disposed of in natural envi-

ronment, the pH reactive binder and the pH buffer solution added to the water disintegratable paper may possibly exert a baneful influence upon natural environment. Moreover, the organic acid contained in the pH buffer solution may possibly change with passage of time, which may possibly have an adverse effect upon the properties of the water disintegratable paper. Still moreover, the water disintegratable paper impregnated with the pH reactive binder is inferior in softness, so that a user cannot use it comfortably. Still 10 moreover, since the pH reactive binder is expensive, the water disintegratable paper impregnated with the pH reactive binder cannot be manufactured at a low cost. Commonly, a water disintegratable sheet is impregnated with a solution of chemicals such as humectant, anti-inflammatory agent, anti-bacterial agent, surfactant, alcohol and perfume, depending on the purpose of the usage. However, if the sheet is impregnated with an inhibitor for inhibiting the pH reactive binder from dissolving, the chemicals must be ones that not react with the inhibitor, so that the selection of chemicals is severely limited.

On the other hand, since the nonwoven sheet disclosed in Japanese Unexamined Patent Publication No. H5-279985 is formed only of the ramie fibers, the ramie fibers are strongly hydrogen bonded to each other. Therefore, the nonwoven sheet becomes stiff without softness, so that a user cannot use the nonwoven sheet comfortably. In addition, Japanese Unexamined Patent Publication No. H5-279985 does not describe water disintegratability of the nonwoven sheet and does not teach how to provide excellent water disintegratability together with improved sheet strength.

### SUMMARY OF THE INVENTION

The present invention has been worked out in view of the 35 shortcoming in the prior art set forth above. It is therefore an object of the present invention to provide a water disintegratable sheet which can offer a good balance of wet and dry strengths and water disintegratability, without exerting a baneful influence upon the human body and environment, and can be manufactured at a low cost, and a method of manufacturing the same.

According to a first aspect of the present invention, there is provided a water disintegratable sheet comprising bast/leaf fibers and at least one kind of primary fibers, wherein

45 the bast/leaf fibers have a Canadian Standard freeness value of at most 600 milliliter and occupy 2 to 75% by weight of a total fiber weight of the sheet.

In detail, the fibers are bonded to each other by means of at least one of:

- 50 (A) entanglement;  
(B) hydrogen bond; and  
(C) Van der Wall's force.

In the water disintegratable sheet of the present invention, the fiber bonding strength is increased by the bast/leaf fibers 55 having a Canadian Standard Freeness value within the above-mentioned range. Therefore, the wet strength and dry strength of the sheet can be increased without any additional binder. When immersed in a large amount of water, on the other hand, the fiber bonding strength due to the bast/leaf fibers is rapidly relieved so that the fibers can be dispersed in water.

In addition, since the water disintegratable sheet contains the primary fibers such as pulp and regenerated cellulose, the fiber bonding strength is prevented from being excessively high, thereby providing soft hand without stiffness.

65 Preferably, the bast/leaf fibers are fibrillated. In this case, mechanical bond due to hydrogen bond and/or Van der

Waals force can easily be caused between the beaten and fibrillated fibers and the primary fibers, resulting in a sheet of high strength.

Preferably, the bast/leaf fibers are leaf fibers. Also preferably, the bast/leaf fibers have a fiber length of at most 20 millimeter. For the bast/leaf fibers, use can be made of at least one of abaca and sisal. The leaf fibers, particularly abaca and sisal, can easily be fibrillated by beating. In addition, these leaf fibers are hardly chopped into small short pieces by beating, while maintaining their fiber strength even after beating. With the fiber length being at most 20 mm, moreover, formation in papermaking process is improved.

Preferably, the primary fibers are biodegradable fibers. If so, when the water disintegratable sheet is disposed of in a toilet or the like, the constituent fibers dispersed in water can be biodegraded. Therefore, the functions of a septic tank and a sewage line will not be damaged, and deterioration of environment can be prevented. In this case, the biodegradable fibers are preferably pulp fibers and/or regenerated cellulose fibers.

Preferably, the water disintegratable sheet has a dry strength of at least 10.0 Newton per 25 millimeter width and a wet strength of at least 1.3 Newton per 25 millimeter width. With the dry strength and wet strength being set within the above-mentioned ranges, the water disintegratable sheet hardly breaks during use.

Preferably, the water disintegratable sheet has a basis weight of 30 to 120 g/m<sup>2</sup>. If the basis weight is less than 30 g/m<sup>2</sup>, sufficient strength cannot be obtained, resulting in breakage during use. If the basis weight is more than 120 g/m<sup>2</sup>, on the other hand, the web formation becomes difficult, causing a variation in properties of the resulting water disintegratable sheet.

Preferably, the water disintegratable sheet has a water disintegrability of at most 300 seconds.

According to a second aspect of the present invention, there is provided a method of manufacturing a water disinTEGRATABLE sheet comprising the steps of:

wet-laying a blend of 2 to 75% by weight of bast/leaf fibers having a Canadian Standard freeness value of at most 600 milliliter and 98 to 25% by weight of at least one kind of primary fibers into a fibrous web; and

drying the fibrous web.

In the present invention, since the bast/leaf fibers having a Canadian Standard Freeness value of at most 600 ml can exhibit a large hydrogen bonding force through the drying step after the wet-laying step, sufficient sheet strength can be obtained in both dry and wet states only with the wet-laying step and the drying step.

If the bast/leaf fibers have a fiber length of at most 20 millimeter, the bast/leaf fibers can be uniformly dispersed in a papermaking process, so that bonds due to the fiber entanglement and/or the hydrogen bond can be uniformly distributed, providing the water disintegratable sheet with excellent formation.

#### BRIEF DESCRIPTION OF THE DRAWINGS

The present invention will be understood more fully from the detailed description given hereinafter and from the accompanying drawings, which, however, should not be taken to be limitative to the invention, but are for explanation and understanding only.

In the drawings:

FIG. 1 is a graph showing fiber length distributions of fibrillated abaca for different Canadian Standard Freeness values; and

5 FIG. 2 is a graph showing fiber length distributions of  
fibrillated lyocell for different Canadian Standard Freeness  
values.

## DESCRIPTION OF THE PREFERRED EMBODIMENT

The term "water disintegrable" as used herein means that when immersed in water, fibers forming a sheet are dispersed in a short period of time so that the sheet breaks into multiple pieces.

The term "web" as used herein means a sheet-like fiber aggregate made by laying down and assembling fibers.

The term "bast/leaf fiber" as used herein means bast fiber or leaf fiber. The bast fiber refers to soft fiber such as flax (linen), ramie, hemp, jute, kenaf and China jute (Indian mallow heapskin). The leaf fiber refers to hard fiber such as abaca, sisal and New Zealand hemp.

The term "primary fiber" as used herein means fiber of the kind different from the bast/leaf fiber.

25 The water disintegratable sheet according to the present invention comprises primary fibers and bast/leaf fibers. The primary fibers and the bast/leaf fibers are wet-laid, and then dried to produce the water disintegratable sheet. The water disintegratable sheet according to the present invention can  
30 be used in a wide variety of applications. For instance, the water disintegratable sheet can be used as a topsheet or backsheets of an absorbent article such as sanitary napkin, vaginal discharge absorbing sheet (panty liner), incontinence pad and disposable diaper or a packaging sheet for  
35 packaging such an absorbent article. It is also possible to use the water disintegratable sheet as dry tissue paper. The water disintegratable sheet may also be used while being impregnated with water or a solution of chemicals. In this case, for instance, the water disintegratable sheet may be used as wet  
40 tissue paper for wiping a human body, or a cleaning sheet for cleaning a toilet or the like.

The bast/leaf fibers used for the water disintegratable sheet of the present invention should have a Canadian Standard Freeness (CSF) value of at most 600 milliliter (ml).

45 The Canadian Standard Freeness value expresses the capacity of fibers to drain water, and also indicates the degree of beating of fibers, wherein low numbers indicate that the fibers are beaten more; high numbers indicate that the fibers are beaten less. When the bast/leaf fibers are so beaten as to obtain a Canadian Standard Freeness value of at most 600 ml, they are fibrillated to provide microfibers. Therefore, the surface area of the bast/leaf fibers is increased due to the microfibers. In addition, physical bonding strength due to entanglement of the microfibers, hydrogen bond and Van der Waal's force can be increased. Should the bast/leaf fibers be unbeaten to have a Canadian Standard Freeness value of more than 600 ml, such bonding strength due to the microfibers can not be obtained.

Although there is no special reason to define the lower limit of the Canadian Standard Freeness value as long as the bast/leaf fibers are fibrillated, the bast/leaf fibers cannot be fibrillated by beating beyond a Canadian Standard Freeness value of about 100 ml. Preferably, the lower limit of the Canadian Standard Freeness value is 200 ml.

65 The beaten bast/leaf fibers preferably have a fiber length of at most 20 millimeter (mm), which refers to a maximum fiber length found in fiber length distribution thereof. If the

fiber length is more than 20 mm, the bast/leaf fibers are hardly uniformly dispersed in a papermaking process, so that bonds due to the entanglement of the bast/leaf fibers and/or the hydrogen bond cannot be uniformly distributed, deteriorating formation. More preferably, the beaten bast/leaf fibers have a fiber length of at most 10 mm. On the other hand, there is no special reason to define the lower limit of the fiber length of the beaten bast/leaf fibers, but 1 mm is appropriate. Since bast/leaf fibers having a fiber length of less than 1 mm easily slip through a mesh screen during the wet-laid process, there is a possibility of decreasing the yield.

Of the bast/leaf fibers, abaca and sisal are most suitable for use in the water disintegratable sheet of the present invention, since the fiber length is from 1.5 to 8.0 mm.

In the present invention, since the bast/leaf fibers are fibrillated, the bast/leaf fibers are bonded to each other or to the primary fibers due to entanglement of the microfibers. In addition, the hydrogen bonding force and Van der Waal's force of the bast/leaf fibers are increased since the surface area of the bast/leaf fibers is increased by beating. That is, the beaten bast/leaf fibers substantially function as a binder to impart strength to the sheet.

The water disintegratable sheet of the present invention should contain 2 to 75% by weight of the bast/leaf fibers, based on the total fiber weight of the water disintegratable sheet in a dry condition. If the bast/leaf fiber content is less than 2% by weight, the force of the bast/leaf fibers for bonding the primary fibers with entanglement, hydrogen bond and so on is weakened, resulting in deterioration of sheet strength. If the bast/leaf fiber content is more than 75% by weight, on the other hand, the hydrogen bonding force between the bast/leaf fibers is excessively increased, so that the resulting water disintegratable sheet becomes stiff, resulting in deterioration of hand and feel with respect to softness.

The term "entangle" as used herein means that fibers (which mainly refer to microfibers of bast/leaf fibers in the present invention) are wrapped and knotted about each other. The term "hydrogen bond" as used herein means a dipole-dipole force between molecules sharing one hydrogen atom, which is covalent bonded to one atom of at least one molecule having strong electronegativity. The term "Van der Waal's force" as used herein means an attraction force between molecules, which corresponds to internal pressure of Van der Waal's equation of state.

Examples of the bast/leaf fibers include flax (linen), ramie, hemp, jute, kenaf, China jute (Indian mallow heapskin), abaca, sisal and New Zealand hemp. In the present invention, a single kind of bast/leaf fibers may be employed alone or two or more kinds of bast/leaf fibers may be employed in combination. The bast/leaf fibers may or may not be bleached. It is, of course, possible to blend bleached bast/leaf fibers with unbleached bast/leaf fibers.

In the present invention, the bast/leaf fibers are beaten and fibrillated. The beaten bast/leaf fiber means that at least a portion of the fiber is split into microfibers. In the present invention, preferably performed is wet beating, in which the bast/leaf fibers can be split into the microfibers while maintaining their original fiber length. However, as long as the Canadian Standard Freeness value is equal to or less than 600 ml, free beating, in which the bast/leaf fibers will be chopped to decrease their fiber length, may also be performed.

For the bast/leaf fibers, as described above, at least one of abaca and sisal is preferably used. Since abaca and sisal are

easy to beat and resulting microfibers are strong, they are suitable for use in the water disintegratable sheet of the present invention.

FIG. 1 shows fiber length distributions of beaten abaca (i.e., how fibers that differ in fiber length are distributed after beating abaca) for different Canadian Standard Freeness values. The fiber length distributions of beaten abaca are plotted with fiber lengths (mm) as abscissa against fiber contents at individual fiber lengths as ordinate. FIG. 2 is for 10 comparison with abaca, and shows fiber length distributions of fibrillated lyocell for different Canadian Standard Freeness values. Here, the fibrillated lyocell was obtained by beating lyocell (purified cellulose fiber) with a refiner.

From FIG. 1, it is seen that the fiber length distribution of 15 beaten abaca is less variable even if the Canadian Standard Freeness i.e., the degree of beating is varied. This means that abaca can easily be fibrillated by beating, and beaten abaca itself is so strong that the split microfibers are hardly 20 chopped into small short pieces even if the beating is further progressed. Here, the individual fiber length distribution curves have their peaks near one half of the maximum fiber length, regardless of the Canadian Standard Freeness values.

When the bast/leaf fibers thus beaten are used, strong 25 microfibers of various fiber lengths increase the fiber bonding strength, resulting in a sheet of high strength. Accordingly, the water disintegratable sheet can be provided with high strength even if the bast/leaf fiber content is not much. By reducing the bast/leaf fiber content as much as possible, softness and improved hand can be provided to the sheet.

On the other hand, as seen from the peaks of fiber length 30 distribution curves of FIG. 2, fibrillated lyocell has a definite main body portion (from which short microfibers protrude) when it is not beaten much, but as the lyocell is beaten more, the main body portion is shortened, and finally, it breaks into 35 multiple short pieces.

From above, it is understood that the bast/leaf fiber is easy 40 to beat as compared with lyocell (purified cellulose fiber) and is prevented from getting too short even if it is beaten much. Thus, since the bast/leaf fiber can easily be fibrillated by beating, it can be used as a low cost material.

The primary fibers are preferably biodegradable. The term 45 "biodegradable" as used herein means that fibers can be broken down in a living body or by bacteria. In this case, since not only the primary fibers but also the bast/leaf fibers are biodegradable, after the water disintegratable sheet is disposed of in a toilet or the like and disintegrated in water, the fibers dispersed in water can be biodegraded. Therefore, the functions of a septic tank and a sewage line will not be 50 damaged, and deterioration of environment can be prevented.

Examples of the primary fiber being biodegradable include natural fiber (except for the bast/leaf fiber) such as 55 pulp fiber, regenerated cellulose fiber and purified cellulose fiber. They may be used alone or in combination.

Examples of regenerated cellulose fiber include viscose rayon (rayon manufactured in viscose process) and cuprammonium rayon (cupra manufactured in cuprammonium process). On the other hand, purified cellulose fiber can be exemplified by lyocell which is manufactured in organic 60 solvent spinning process. Such cellulose fibers may be fibrillated.

Examples of pulp fiber include wood pulp such as 65 bleached softwood pulp, cotton linter pulp and mercerized pulp. They may be bleached or unbleached chemical pulp. It is, of course, possible to blend bleached chemical pulp with unbleached chemical pulp. Here, they may or may not be beaten, and may or may not be fibrillated. However, it is

preferred that the pulp fibers are beaten to have a Canadian Standard Freeness value of 650 to 300 ml.

The primary fibers preferably have a fiber length of at most 20 mm. Here, the pulp fibers have a fiber length of about 1 to 4 mm from the beginning. On the other hand, the fiber length of the regenerated cellulose fibers is preferably set at 20 mm or less. If the fiber length is more than 20 mm, the formation after papermaking will be deteriorated, as described above.

The primary fibers, particularly the regenerated cellulose fibers, preferably have a fineness of 0.6 to 11 dtex. If the fineness is less than 0.6 dtex, such thin fibers are hardly disentangled when immersed in water, resulting in deterioration of water disintegratability. If the fineness is more than 11 dtex, on the other hand, the sheet surface becomes rough, resulting in deterioration of feel.

As has been described above, the water disintegratable sheet of the present invention contains 2 to 75% by weight of bast/leaf fibers. Therefore, the content of the primary fibers such as regenerated cellulose fibers, purified cellulose fibers and pulp fibers is 25 to 98% by weight.

The water disintegratable sheet of the present invention can be manufactured as follows.

At first, using a cylinder machine, "tan-ami" (short wire) machine, inclined wire machine or Fourdrinier machine, the bast/leaf fibers and the primary fibers suspended in water are fed onto a cylinder mold or the like, and collected thereon to form a fibrous web. Then, the fibrous web is transferred onto a felt belt of high surface density, and conveyed while being wrapped around a dry drum for drying.

In the completed water disintegratable sheet, the microfibers of the bast/leaf fibers are entangled about the primary fibers, and exhibit the hydrogen bond and the bonding force due to the Van der Waal's force. Thus, the sheet strength can be maintained high. Here, it should be noted that any mechanical force for entangling fibers is not applied to the fibrous web after the wet-laid process. That is, the water disintegratable sheet of the present invention is not subjected to a water-jet treatment or the like.

The water disintegratable sheet preferably has a wet strength of at least 1.3 Newton (N) per 25 millimeter (mm) width, wherein the sheet is impregnated with water twice as heavy as the sheet weight. In a state where the sheet is dried, on the other hand, the water disintegratable sheet preferably has a dry strength of at least 10.0 N per 25 mm width.

Here, the wet and dry strengths refer to the square root of the product of the tensile strength (breaking strength) in MD and the tensile strength (breaking strength) in CD, wherein MD is a traveling direction of the web in the manufacturing process and CD is a direction perpendicular to MD.

When the water disintegratable sheet is disposed of in a flush toilet and immersed in a large amount of water in a flush toilet or a septic tank, the microfibers of the bast/leaf fibers can be disentangled and their hydrogen bonding force can be weakened. Moreover, the Van der Waal's force can be weakened by the flow of water. Therefore, the fibers can be dispersed in water.

The water disintegratable sheet preferably has a water disintegratability (water disintegration time) of at most 300 seconds. If the water disintegratability is equal to or less than 300 seconds, a used sheet disposed of in a toilet or the like can be effectively prevented from floating and remaining in a septic tank. More preferably, the water disintegratability is at most 100 seconds. If it is equal to or less than 100 seconds, the water disintegratable sheet disposed of in a flush toilet can be disintegrated to some extent before it reaches a septic tank.

The water disintegratable sheet preferably has a basis weight of 30 to 120 g/m<sup>2</sup>. If the basis weight is less than 30 g/m<sup>2</sup>, sufficient strength cannot be obtained, so that the sheet may easily break during use. If the basis weight is more than 100 g/m<sup>2</sup>, it takes long time for the sheet to disintegrate in water, deteriorating water disintegratability. In addition, if the basis weight is more than the limit, it is difficult to provide a web with a uniform fiber density, causing a variation in properties such as strength and water disintegratability. However, in case where two or more water disintegratable sheets are to be stacked one on another for use, the basis weight of each water disintegratable sheet may be less than 30 g/m<sup>2</sup>.

The water disintegratable sheet of the present invention may be used as a cleaning article such as wet tissue paper or wet wiper, which is to be supplied to consumers while being impregnated with a liquid. In this case, the water disintegratable sheet is impregnated with a liquid, which may be purified water, but may also contain humectant, anti-inflammatory agent, anti-bacterial agent, surfactant, alcohol, perfume and so on, according to demand. Here, it should be noted that since the water disintegratable sheet of the present invention is not impregnated with any inhibitor for inhibiting an organic substance binder from dissolving, the selection of chemicals to be added to the water disintegratable sheet depending on the purpose of the usage is not severely limited.

The water disintegratable sheet of the present invention may be of multi-layer structure. Such multi-layer structure can be obtained using any one of the foregoing paper machines. For example, a first web is wet-laid on the inclined wire or the like, and a second web is further wet-laid on the first web, to thereby form a multi-layer web. Such process may be repeated according to demand. In this case, the blending ratio of the bast/leaf fibers and the primary fibers may vary for different webs.

As has been described hereinabove, the water disintegratable sheet of the present invention is not impregnated with either an organic substance binder such as pH reactive binder or a pH buffer solution containing an organic acid, but the bast/leaf fibers function as binder. Therefore, it never exerts a baneful influence upon the human body and environment. In addition, the properties of the water disintegratable sheet hardly change with passage of time, because the sheet does not contain the pH buffer solution of which the organic acid changes with passage of time. Moreover, since no organic substance binder is added, the water disintegratable sheet can be made soft to the touch, so that the sheet can be comfortably used.

## EXAMPLES

### Manufacturing Conditions of Examples and Comparative Examples

For preparing Examples and Comparative Examples, fibers were blended in ratios shown in Tables 1 to 5, and suspended in water to obtain fiber suspension. At this time, the fiber content was set at 0.02% by weight, based on the weight of the fiber suspension. Then, the fibers suspended in water were collected on a papermaking wire of 90 meshes, to thereby form a fibrous web having a length of 25 cm and a width of 25 cm. Thereafter, the web was dried by heating it for 90 seconds at 150° C. with a rotary drum type dryer to obtain Examples and Comparative Examples.

## Used Fibers of Examples and Comparative Examples

As the bast/leaf fibers, used was abaca (Grade: JK). The abaca was suspended in water to have a fiber concentration of 0.6% by weight, and beaten with a mixer to have various Canadian Standard Freeness values, as shown in Tables 1 to 5. The fiber length distributions of the used abaca for respective Canadian Standard Freeness values were shown in FIG. 1.

As primary fibers, used were bleached softwood kraft pulp (NBKP), rayon and fibrillated lyocell.

The bleached softwood kraft pulp was beaten with a double disc refiner (of which two discs were rotated in opposite directions for beating) to have a Canadian Standard Freeness value of 600 ml.

The rayon (regenerated cellulose fiber) had a fineness of 1.1 dtex and a fiber length of 5 mm, which was manufactured by Daiwabo Rayon, Japan (trade name: Corona).

The fibrillated lyocell shown in Table 5 was prepared by beating lyocell (purified cellulose fiber having a fineness of 1.7 dtex and a fiber length of 6 mm) with a refiner to have a Canadian Standard Freeness value of 200 ml.

## (Method for Measuring Basis Weight and Thickness)

Basis weights and thicknesses of Examples and Comparative Examples were measured after standing for at least 30 minutes in an atmosphere having a temperature of  $20\pm2^\circ\text{C}$ . and a relative humidity of  $65\pm2\%$ .

## (Method for Measuring Canadian Standard Freeness)

Canadian Standard Freeness was measured using a Canadian Standard Freeness tester composed of a filter cartridge, a measuring funnel and a table supporting the filter cartridge and the funnel. At the bottom of the filter cartridge, there was disposed a metal sieve plate, which was a circular plate having a diameter of  $111.0\pm0.5$  mm and a thickness of 0.5 mm and having 97 apertures per  $1\text{ cm}^2$ . Each aperture had a diameter of 0.50 mm. The measuring funnel was made of metal, and had a diameter of 204 mm at its upper opening and an entire length of about 277 mm. This measuring funnel was provided with a bottom orifice and a side pipe.

The bottom orifice was provided at the bottom of the measuring funnel, and had a minimum diameter of  $3.05\pm0.01$  mm. The bottom orifice was designed to discharge  $530\pm5$  ml of water per minute, when water at  $20.0\pm0.5^\circ\text{C}$ . was supplied to the measuring funnel at a rate of  $725\pm25$  ml per minute. At this time, water that overflowed was intended to flow from the side pipe. The side pipe was a hollow tube having an internal diameter of about 13 mm and penetrating the side of the measuring funnel. The penetration length was adjustable. The volume of water between the upper portion of the bottom orifice and the overflow water-level was  $23.5\pm0.2$  ml.

The fibers were completely dispersed in water to a fiber concentration of 0.3% by weight, to thereby produce a sample liquid at  $20.0\pm0.5^\circ\text{C}$ . Then, 1000 ml of sample liquid was gently put in the filter cartridge to flow down to the measuring funnel, and an amount of water discharged from the side pipe was measured. The thus-measured value was rounded to an integral number, and the resulting numerical number was taken as a value of Canadian Standard Freeness, indicating the numerical number together with "CSF".

## (Method of Measuring Wet Strength)

A test piece having a size of  $25\times150$  mm, of which the short side was extended along CD and the long side was extended along MD, and a test piece having a size of  $25\times150$  mm, of which the short side was extended along MD and the long side was extended along CD, were prepared, impregnated with a distilled water twice as heavy as each test piece, sealed in a plastic bag, and allowed to stand for 24 hours in an atmosphere having a temperature of  $20\pm2^\circ\text{C}$ . Then, the test pieces were taken out, and the short sides of each test piece were held with chucks of a tension tester. The initial chuck-to-chuck distance was set at 100 mm, and a tensile test was performed at a tension speed of 100 mm/minute. The maximum load (breaking load) measured by the tester was taken as a measured value. Such tensile test was performed both for the test piece having the long side along MD and the test piece having the long side along CD.  $\sqrt{(\text{measured value in MD})\times(\text{measured value in CD})}$  was taken as the wet strength.

## (Method of Measuring Dry Strength)

A test piece having a size of  $25\times150$  mm, of which the short side was extended along CD and the long side was extended along MD, and a test piece having a size of  $25\times150$  mm, of which the short side was extended along MD and the long side was extended along CD, were prepared, and the short sides of each test piece were held with chucks of a tension tester. The initial chuck-to-chuck distance was set at 100 mm, and a tensile test was performed at a tension speed of 100 mm/minute. The maximum load (breaking load) measured by the tester was taken as a measured value. Such tensile test was performed both for the test piece having the long side along MD and the test piece having the long side along CD.  $\sqrt{(\text{measured value in MD})\times(\text{measured value in CD})}$  was taken as the dry strength.

## (Method for Measuring Water Disintegration Time)

A disc rotor having a diameter of 35 mm and a thickness of 12 mm was put in a 300 ml beaker, which was filled with 300 ml of ion exchanged water and put on a magnetic stirrer. Then, the ion exchanged water was stirred by driving the rotor to rotate at a rate of 600 rpm. During stirring, a water disintegratable sheet cut into a size of  $10\text{ cm}\times10\text{ cm}$  was put in the ion exchanged water, thereby making the constituent fibers of the water disintegratable sheet disperse in the ion exchanged water. The time required for the fibers to disperse since the water disintegratable sheet was put in the ion exchanged water was measured by visual observation with a stop water. The time thus measured was taken as the water disintegration time.

## (Abaca Content)

Table 1 shows relationships between the abaca content and the dry and wet strengths.

From Table 1, it is seen that the dry strength and wet strength can be increased by increasing the abaca content.

It should be noted that the water disintegratable sheet of the present invention preferably has a wet strength of at least 1.3 N/25 mm, since the sheet will easily break in actual use if the wet strength is less than 1.3 N/25 mm. From Table 1, it is seen that the abaca content should be 2.0% or more in order to obtain a wet strength of 1.3 N/25 mm or more.

TABLE 1

|                           |                        | Com.             | Ex. 1 | Ex. 1 | Ex. 2 | Ex. 3 | Ex. 4 | Ex. 5 | Ex. 6 | Ex. 7 | Ex. 8 | Com.  | Ex. 2 |
|---------------------------|------------------------|------------------|-------|-------|-------|-------|-------|-------|-------|-------|-------|-------|-------|
| Constituent               | NBKP (600 mlCSF)       | wt. %            | 85.0  | 83.0  | 82.0  | 80.0  | 70.0  | 55.0  | 50.0  | 35.0  | 10.0  | 0.0   |       |
| Fiber and                 | Rayon (1.1 dtex, 5 mm) | wt. %            | 15.0  | 15.0  | 15.0  | 15.0  | 15.0  | 15.0  | 15.0  | 15.0  | 15.0  | 15.0  | 0.0   |
| Content                   | Abaca (200 mlCSF)      | wt. %            | 0.0   | 2.0   | 3.0   | 5.0   | 15.0  | 30.0  | 35.0  | 50.0  | 75.0  | 100.0 |       |
| Basis Weight              |                        | g/m <sup>2</sup> | 50.0  | 50.0  | 50.0  | 50.0  | 50.0  | 50.0  | 50.0  | 50.0  | 50.0  | 50.0  | 50.0  |
| Thickness                 |                        | mm               | 0.20  | 0.19  | 0.19  | 0.20  | 0.19  | 0.21  | 0.20  | 0.20  | 0.20  | 0.20  | 0.17  |
| Dry Strength              |                        | N/25 mm          | 44.59 | 47.75 | 49.68 | 52.14 | 55.49 | 57.17 | 59.11 | 63.21 | 65.11 | 84.23 |       |
| Wet Strength              |                        | N/25 mm          | 1.18  | 1.52  | 1.62  | 1.70  | 2.01  | 2.30  | 2.40  | 2.51  | 2.77  | 3.51  |       |
| Water Disintegration Time |                        | second           | 19    | 20    | 22    | 22    | 21    | 22    | 23    | 25    | 25    | 27    |       |

(Canadian Standard Freeness of Abaca)

15

Table 2 shows relationships between Canadian Standard Freeness (degree of beating) of abaca and the dry strength and wet strength.

From Table 2, it is seen that as the Canadian Standard Freeness value of abaca is decreased (as abaca is beaten more), the dry strength and wet strength are increased. It is also seen that abaca having a Canadian Standard Freeness value of 600 ml or less should be contained in order to obtain a wet strength of 1.3 N/25 mm or more.

TABLE 2

|                           |                        | Com.             | Ex. 3 | Ex. 9 | Ex. 10 | Ex. 11 |
|---------------------------|------------------------|------------------|-------|-------|--------|--------|
| Constituent               | NBKP (600 mlCSF)       | wt. %            | 80.0  | 80.0  | 80.0   | 80.0   |
| Fiber and                 | Rayon (1.1 dtex, 5 mm) | wt. %            | 15.0  | 15.0  | 15.0   | 15.0   |
| Content                   | Abaca (unbeaten)       | wt. %            | 5.0   | —     | —      | —      |
|                           | Abaca (600 mlCSF)      | wt. %            | —     | 5.0   | —      | —      |
|                           | Abaca (400 mlCSF)      | wt. %            | —     | —     | 5.0    | —      |
|                           | Abaca (200 mlCSF)      | wt. %            | —     | —     | —      | 5.0    |
| Basis Weight              |                        | g/m <sup>2</sup> | 50.0  | 50.0  | 50.0   | 50.0   |
| Thickness                 |                        | mm               | 0.20  | 0.21  | 0.20   | 0.20   |
| Dry Strength              |                        | N/25 mm          | 43.21 | 47.93 | 50.17  | 52.14  |
| Wet Strength              |                        | N/25 mm          | 1.11  | 1.38  | 1.51   | 1.70   |
| Water Disintegration Time |                        | second           | 18    | 19    | 20     | 22     |

(Fiber Length of Rayon)

Table 3 shows relationships between the fiber length of rayon (regenerated cellulose fiber) and the dry and wet strengths. From Table 3, it is seen that as the fiber length of rayon is increased, the dry strength and wet strength are increased, and that if the fiber length of rayon is 20 mm or less, a good balance of the strength and the water disintegrability can be obtained.

TABLE 3

|                           |                         | Ex. 12           | Ex. 13 | Ex. 14 | Ex. 15 |
|---------------------------|-------------------------|------------------|--------|--------|--------|
| Constituent               | NBKP (600 mlCSF)        | wt. %            | 80.0   | 80.0   | 80.0   |
| Fiber and                 | Abaca (200 mlCSF)       | wt. %            | 5.0    | 5.0    | 5.0    |
| Content                   | Rayon (1.1 dtex, 5 mm)  | wt. %            | 15.0   | —      | —      |
|                           | Rayon (1.1 dtex, 7 mm)  | wt. %            | —      | 15.0   | —      |
|                           | Rayon (1.1 dtex, 10 mm) | wt. %            | —      | —      | 15.0   |
|                           | Rayon (1.1 dtex, 12 mm) | wt. %            | —      | —      | —      |
| Basis Weight              |                         | g/m <sup>2</sup> | 50.0   | 50.0   | 50.0   |
| Thickness                 |                         | mm               | 0.20   | 0.21   | 0.20   |
| Dry Strength              |                         | N/25 mm          | 52.14  | 53.94  | 54.10  |
| Wet Strength              |                         | N/25 mm          | 1.70   | 1.84   | 2.01   |
| Water Disintegration Time |                         | second           | 22     | 19     | 19     |

## 13

(Basis Weight of Water Disintegratable Sheet)

Table 4 shows relationships between the basis weight of the water disintegratable sheet and the dry strength, wet strength and water disintegration time.

From Table 4, it is seen that the dry strength and wet strength can be increased by increasing the basis weight. The basis weight should be 30 g/m<sup>2</sup> or more in order to obtain a wet strength of 1.3 N/25 mm or more.

## 14

out any pH reactive binder. In addition, since neither an organic substance binder nor a pH buffer solution containing an organic acid is required, the sheet never exerts a baneful influence upon the human body and environment, and the properties of the water disintegratable sheet hardly change with passage of time. Moreover, the water disintegratable sheet can be made soft to the touch, so that the sheet can be comfortably used. Still moreover, the selection of chemicals

TABLE 4

|                           |                        | Com. Ex. 4       | Com. Ex. 5 | Ex. 16 | Ex. 17 | Ex. 18 | Ex. 19 | Ex. 20 | Ex. 21 |
|---------------------------|------------------------|------------------|------------|--------|--------|--------|--------|--------|--------|
| Constituent               | NBKP (600 mlCSF)       | wt. %            | 80.0       | 80.0   | 80.0   | 80.0   | 80.0   | 80.0   | 80.0   |
| Fiber and Content         | Rayon (1.1 dtex, 5 mm) | wt. %            | 15.0       | 15.0   | 15.0   | 15.0   | 15.0   | 15.0   | 15.0   |
| Basis Weight              | Abaca (200 mlCSF)      | wt. %            | 5.0        | 5.0    | 5.0    | 5.0    | 5.0    | 5.0    | 5.0    |
| Thickness                 |                        | g/m <sup>2</sup> | 15.0       | 20.0   | 30.0   | 40.0   | 50.0   | 70.0   | 100.0  |
| Dry Strength              |                        | mm               | 0.08       | 0.10   | 0.14   | 0.17   | 0.20   | 0.29   | 0.39   |
| Wet Strength              |                        | N/25 mm          | 12.33      | 19.45  | 33.94  | 45.32  | 52.14  | 54.98  | 55.73  |
| Water Disintegration Time |                        | N/25 mm          | 0.55       | 0.70   | 1.44   | 1.58   | 1.70   | 2.58   | 3.28   |
|                           |                        | second           | 11         | 19     | 20     | 22     | 30     | 32     | 34     |

(Comparison of Abaca Versus Fibrillated Lyocell With Respect to Dry Strength and Wet Strength)

Table 5 shows how the dry strength and wet strength vary between abaca and fibrillated lyocell having the same Canadian Standard Freeness value, while the abaca content is changed.

From Table 5, it is seen that when abaca is compared with fibrillated lyocell having the same Canadian Standard Freeness value, similar dry and wet strengths can be obtained even if the abaca content is smaller than the fibrillated lyocell content.

to be added to the water disintegratable sheet is not severely limited, and the production cost can be reduced.

Although the present invention has been described with respect to exemplary embodiments thereof, it should be understood by those skilled in the art that the foregoing and various other changes, omission and additions may be made therein and thereto, without departing from the spirit and scope of the present invention. Therefore, the present invention should not be understood as limited to the specific embodiments set out above but to include all possible

TABLE 5

|                           |                                 | Ex. 2            | Ex. 11 | Com. Ex. 6 |
|---------------------------|---------------------------------|------------------|--------|------------|
| Constituent               | NBKP (600 mlCSF)                | wt. %            | 82.0   | 80.0       |
| Fiber and Content         | Rayon (1.1 dtex, 5 mm)          | wt. %            | 15.0   | 15.0       |
|                           | Abaca (200 mlCSF)               | wt. %            | 3.0    | 5.0        |
| Basis Weight              | Fibrillated lyocell (200 mlCSF) | wt. %            | —      | 5.0        |
| Thickness                 |                                 | g/m <sup>2</sup> | 50.0   | 50.0       |
| Dry Strength              |                                 | mm               | 0.19   | 0.20       |
| Wet Strength              |                                 | N/25 mm          | 49.68  | 52.14      |
| Water Disintegration Time |                                 | N/25 mm          | 1.62   | 1.70       |
|                           |                                 | second           | 22     | 22         |
|                           |                                 |                  |        | 33         |

As has been described hereinabove, the water disintegratable sheet of the present invention can achieve a good balance of sheet strength and water disintegratability with-

65 embodiments which can be embodied within a scope encompassed and equivalent thereof with respect to the feature set out in the appended claims.

**15**

What is claimed is:

1. A water disintegratable sheet comprising at least one kind of primary fibers and leaf fibers selected from the group consisting of abaca and sisal, wherein  
the leaf fibers are beaten and fibrillated to have a Canadian Standard Freeness value of at most 600 milliliters and occupy 2 to 75% by weight of a total fiber weight of the sheet to thereby achieve a water disintegratability of at most 300 seconds, and a length of the fibrillated leaf fibers is 1.5 mm to 8 mm.
2. The water disintegratable sheet as set forth in claim 1, wherein the sheet has a dry strength of at least 10.0 Newton per 25 millimeter width and a wet strength of at least 1.3 Newton per 25 millimeter width.

**16**

3. The water disintegratable sheet as set forth in claim 2, wherein the leaf fibers have a Canadian Standard Freeness value of 200 to 600 milliliters and have a water disintegratability of at most 100 seconds.
4. The water disintegratable sheet as set forth in claim 3, wherein the primary fibers are at least one of wood pulp fibers and regenerated cellulose fibers.
5. The water disintegratable sheet as set forth in claim 4, wherein the wood pulp fibers have a Canadian Standard Freeness value of 300 to 650 milliliters.
6. The water disintegratable sheet as set forth in claim 4, wherein the regenerated cellulose fibers have a fineness of 0.6 to 11 dtex and a length of at most 20 millimeters.

\* \* \* \* \*